

# UNITED STATES PATENT OFFICE.

FRANK E. COOMBS, OF AU SABLE FORKS, NEW YORK.

## PROCESS OF REMOVING SCALE.

1,049,054.

No Drawing.

Specification of Letters Patent. Patented Dec. 31, 1912.

Application filed July 8, 1911. Serial No. 637,440.

To all whom it may concern:

Be it known that I, FRANK E. COOMBS, a citizen of the United States, residing at Au Sable Forks, in the county of Essex and 5 State of New York, have invented certain new and useful Improvements in Processes of Removing Scale, of which the following is a specification.

This invention relates to processes of 10 moving scale; and it comprises a method wherein scaled surfaces of boilers, evaporators, vacuum pans, grainers, heaters, etc., which are advantageously first cleansed with water or the like, are treated with a 15 solution of caustic soda at a temperature above 100° C. (212° F.) to produce a disintegration of the scale, such solution being advantageously filmed or otherwise distributed over the scale, and the scale is there- 20 after removed, the soda being, if desired, regained for subsequent use; all as more fully hereinafter set forth and as claimed.

In the operation of many heat-transferring liquid-treating devices, such as evaporating pans, vacuum pans, boilers, grainers, heaters, etc., the surface exposed to the liquid after a time scales up, much impeding transference of heat. The scale is usually composed of or comprises calcium salts, such 25 as the carbonate, sulfate, sulfite, citrate, acetate, etc., the particular acid or acids combined with the calcium varying with the liquid treated; and it often also contains various mechanical and other impurities 30 such as mud, iron salts, alumina compounds, silica and silicates, sticks, straws, sand, etc. With boilers, ordinarily the scale is largely carbonate or sulfate; with waste sulfite liquors and the like it may be largely sulfite; 35 with sugar juices it may be all these salts and also calcium salts of organic acids, etc.

The scale is often firmly adherent and as in modern heat transferring devices, the heating surfaces are relatively large and are 45 hard to get at, its removal is difficult. This is particularly the case where, as in many types of evaporators, the heating and evaporating of the liquid takes place from the external surface of tubes of relatively small 50 diameter. Scale forming on the outside of such tubes is difficult to remove, owing to the lack of room between the closely set tubes and the consequent impracticability of reaching their external surfaces with scraping tools.

In the prior art many attempts have been

made to remove scale with one solution or another, but without any great degree of success. Its removal is usually an expensive and tedious operation, often requiring the 60 apparatus to be shut down for a long period of time and to be more or less dismantled. With any amount of scale on the heat transferring surfaces the efficiency goes down very markedly. Often mechanical means of 65 one type or another, such as scrapers, brushes or the like are employed in removing scale but it is difficult to prevent mechanical injury thereby and particularly where the heat transferring element is, as is 70 frequently the case, of copper; copper being a relatively soft metal.

In the present invention I have devised a simple, cheap, ready and rapid method of 75 solubilizing or disintegrating and removing scale from evaporating surfaces, based on the fact of a reversal of the action of soda upon lime or calcium salts occurring when a caustic soda solution is above 1.10 sp. g. and 80 100° C. (212° F.). At most ordinary densities and temperatures the action of lime upon a soda salt of an acid forming an insoluble calcium salt is to form such a salt and to set free caustic soda. For example, 85 quicklime with a solution of sodium carbonate forms calcium carbonate and free caustic soda; this being the ordinary method of making caustic soda from carbonate. With sodium sulfate, the reaction, though not so ready, tends to go in the same direction. If, 90 however, insoluble calcium compounds, such as the carbonates or sulfates be treated with a caustic soda solution at a temperature above 100° C. and with a relatively strong soda solution, the reaction goes in the reverse 95 direction, the calcium salts being converted into more or less soluble sodium salts. The strength of the soda solution in contact with the scaled surface should be at least 12° to 13° Bé. (1.091-1.10 specific gravity) and is 100 best about 30° Bé. or higher. With a weak soda solution it is particularly advantageous to perform the scale-disintegrating action at a temperature above the normal boiling point of the liquid, the liquid being heated 105 under pressure. Caustic soda solutions of less than about 1.10 specific gravity even at their boiling points affect many scale-forming materials to only a slight degree. With a stronger hot soda solution, scale removal 110 may be performed at the ordinary atmospheric pressure. It is also best to present

the soda solution to the surface in a relatively subdivided form as by spraying or traversing it along the scaled surface in a relatively thin film or layer. With modern 5 filming evaporators or vacuum pans this subdivision offers no difficulties. The same is true of many of the flash types of boilers or evaporators.

Before treatment with the soda, the 10 scaled surface is preferably thoroughly cleansed by treatment with water or steam to remove soluble bodies, since the solution of these soluble bodies in the soda lye, which is usually to be recovered and used again, is 15 disadvantageous. After the treatment the scale will be disintegrated and may be removed with acids or mechanically, as by forcible impingement of jets of water against the incrusted surface, or by the 20 usual forms of stiff brushes or scrapers, or by other chemical or mechanical means, or by both chemical and mechanical means. The action of the soda is to convert the lime salts into new forms, the corresponding 25 acids of the original lime salts dissolving in the soda to a greater or less extent and this action is accompanied by disintegration or loosening of the scale. And the higher temperatures have the further merit of more 30 rapidly attacking many organic bodies which are present, and which act as a cement among the various layers of the scale, which has always a laminated structure. After the soda treatment, the scaled surface 35 should of course be washed to recover any adhering soda. Very frequently this washing operation alone suffices to remove the scale. The washing operation is best done with hot water.

40 The means to be employed for producing contact between soda and scale during the disintegration treatment may be as desired and will vary with the particular apparatus to be treated. As stated, it is best to use the 45 soda solution in subdivided form, as this gives a better action, but the scaled surface may be submerged in the soda if desired. This however involves the use of relatively large amounts of soda; neither is 50 the action so quick. In the case of a film evaporator, the soda solution may be simply caused to follow the usual path of liquid through the apparatus to be treated. As film evaporators are ordinarily constructed 55 to work under vacuum, *i. e.* at a relatively low heat, it is necessary in cleaning them to use either a strong soda solution, as one of 25 B., or with a weaker one of about 13 B., to arrange the valves, etc., so as to allow 60 performing the treatment under some pressure. With other types of apparatus, the soda solution may be sprayed or filmed over the heat transferring surface by any appropriate means.

65 I have found that this method is par-

ticularly applicable to the treatment of scaled evaporating elements of the climbing film type of evaporator. In these evaporators, evaporation is performed interiorly of relatively long and narrow tubes, the interior of which is rather inaccessible; and where such evaporators are employed for treating rapidly scaling liquids, such as waste sulfite liquor, the use of the present invention is particularly advantageous. In 70 modern practice (see Patent 833,634) sulfite waste liquor coming from paper pulp digesters is carefully neutralized with lime or dolomitic lime and evaporated to a thick liquor of about 30 B. As the liquor contains some sulfites and sulfates and some are formed by this neutralization step, there is apt to be a deposit of hard, clinging scale in treating the neutralized liquid. The present process is particularly adapted for 75 removing scale formed from such liquids treated in this type of apparatus.

The caustic soda solution may be passed over the scaled surface one or more times. Ordinarily in order to economize solutions 90 it is better to pass the soda over the scaled surface a plurality of times. With film evaporators this can readily be done. Where the soda is circulated through the apparatus cyclically and where evaporation is allowed 95 to take place in the apparatus, it may be necessary to add water to the system at some point to replace evaporation losses and preserve the desired density. After treatment of the scale from the apparatus, the 100 soda is contaminated by dissolved salts of the acids removed from the scale, such as sulfates, sulfites, carbonates, etc., and in order to regain the soda in active form, the solution must be suitably treated. The best 105 method of doing this is to add water to reduce the specific gravity below 1.10 and then treat with quicklime. The reduction of specific gravity causes precipitation of lime salts insoluble in caustic soda solutions 110 of less than 1.10 specific gravity, in so far as such salts or their acids have been dissolved, with accompanying regeneration of part of the caustic soda. The addition of quicklime completes the precipitation of insoluble lime salts and recovers all the remaining caustic soda. The lime is best used as quicklime since the heat of hydration materially assists in causing the desired reactions. The regenerated soda solution so 115 produced is too dilute for the present purposes but it may be readily brought up to the density desired by allowing evaporation to the desired extent during the use of the solution in the scale removing operation.

120 After cleansing an evaporator with soda solution, the latter may be treated with lime in the described manner and the mixture allowed to stand until the solution is again required. The solution may then be drawn 130

off from the lime, and circulated through the boiler or evaporator to be cleansed, thereby causing sufficient evaporation to bring it back to its original strength. New 5 caustic soda may be added when necessary. The lime mud may be washed to regain caustic soda or it may be sent to waste.

In circulating relatively small quantities of scale-removing solution over evaporating 10 surfaces, there is usually more or less loss of water by evaporation. Concentration of the solution due to this cause may be prevented from occurring to an undesirable extent by providing means for automatically 15 supplying water to the caustic solution at any convenient point in its circulation, as by means of a ball-cock or float valve.

While I have described more particularly 20 the use of a solution of caustic soda, regarding such caustic soda solution as particularly advantageous for the present purposes, yet I may use a solution of sodium carbonate under heat and pressure. With 25 a hot solution of sodium carbonate under pressure the disintegrating action upon scale is much more pronounced than where such solution is used under less pressure or at a less temperature. I may therefore use carbonate of soda circulated through 30 the evaporating apparatus to be cleansed in the same manner as caustic soda, using a strong solution and finely dividing it over the scale surfaces, as by filming it thereon or spraying it thereover. In cleansing 35 vacuum apparatus with a sodium carbonate solution, the solution may be caused to follow the normal course of liquid to be evaporated through the apparatus, but the apparatus should preferably, instead of being 40 worked under vacuum, be worked under pressure. It is best to use a sodium carbonate solution relatively strong and to cause the heat to be above the normal boiling point of the solution used under atmospheric pressure. 45

While caustic potash and potassium carbonate may be employed in lieu of caustic soda or sodium carbonate, they are more expensive and ordinarily offer no special advantage over soda. As, however, the solutions may be regained, the item of additional expense is not very great.

What I claim is:—

1. In removing scale from evaporating 55 elements, the process which comprises subjecting the scaled evaporative surfaces of such elements to the action of a heated solution of caustic soda at a temperature above 100° C. and of a density above 1.10 60 specific gravity.

2. In removing scale from evaporating elements, the process which comprises subjecting the scaled evaporative surfaces of

such elements to the action of a heated solution of caustic soda of a density exceeding 6 1.10 specific gravity.

3. In removing scale from evaporative surfaces, the process which comprises washing the scaled surfaces to remove soluble matters, subjecting the washed surfaces to 7 the action of a heated solution of caustic soda at a temperature above 100° C., and thereafter removing the softened scale.

4. In removing scale from evaporative surfaces, the process which comprises 7 treating the scaled surfaces with water to remove soluble matters, subjecting the washed surfaces to the action of a heated solution of caustic soda of a density exceeding 1.10 specific gravity and thereafter removing the softened scale. 8

5. In removing scale from evaporative surfaces, the process which comprises water treatment of the surfaces to remove soluble matters, subjecting the washed surfaces to 8 the action of a heated solution of caustic soda of a density exceeding 1.10 specific gravity and at a temperature above 100° C., and thereafter removing the softened scale. 9

6. In removing scale from evaporating 9 surfaces, the process which comprises treating such surfaces with a traveling film of alkali solution at a density above 1.10 specific gravity.

7. In removing scale from evaporating 9 surfaces, the process which comprises treating such surfaces with a traveling film of caustic soda solution of not less than about 1.10 specific gravity and at a temperature above 100° C. 1

8. In removing scale from evaporating surfaces, the process which comprises treating such surfaces with a solution of caustic alkali of a density above 1.10 specific gravity and heating the alkali solution 1 under pressure while in contact with said surfaces to a temperature above the normal boiling point of said alkali solution.

9. In removing scale from evaporating surfaces, the process which comprises treating such surfaces with an alkaline solution of above 1.10 specific gravity and heating such solution under pressure while in contact with said surfaces to a temperature above the boiling point of said solution. 1

10. In removing scale from evaporating surfaces, the process which comprises circulating a heated solution of a caustic alkali in relatively thin layers over such surfaces.

In testimony whereof, I affix my signature in the presence of two subscribing witnesses. 1

FRANK E. COOMBS.

Witnesses:

L. C. BOLLES,  
JAS. A. SHIRRAS.